

F. G. PERKINS, DEC'D.  
G. S. PERKINS, EXECUTRIX,  
PROCESS OF MAKING GLUE.  
APPLICATION FILED DEC. 26, 1913.

1,351,275.

Patented Dec. 25, 1917.



WITNESSES

J. O. Temple  
G. M. Morris.

Frank G. Perkins, d.b.  
INVENTOR  
Gertude S. Perkins, Executrix

BY  
Kingsley Kenyon  
ATTORNEYS

# UNITED STATES PATENT OFFICE.

FRANK G. PERKINS, DECEASED, LATE OF LANSDALE, PENNSYLVANIA, BY GERTRUDE S. PERKINS, EXECUTRIX, OF SOUTH BEND, INDIANA, ASSIGNOR TO PERKINS GLUE COMPANY, A CORPORATION OF PENNSYLVANIA.

## PROCESS OF MAKING GLUE.

1,251,275.

Specification of Letters Patent. Patented Dec. 25, 1917.

Application filed December 26, 1913. Serial No. 808,739.

To all whom it may concern:

Be it known that FRANK G. PERKINS, deceased, late of Lansdale, borough of Lansdale, State of Pennsylvania, did invent certain new and useful Improvements in Processes of Making Glue, of which the following is a specification.

The invention relates to processes of making glue in a jacketed kettle from starch, water and solvent for the starch, and is especially adapted to the making of vegetable joiner's glue in accordance with U. S. reissued Letters Patent No. 13486 of July 2, 1912. In said reissued Letters Patent it is 10 stated that temperature affects the amount of solvent necessary to change the starch glue base into a glue suitable for joinery and that at successively increasing temperatures one is enabled to bring across the mixture or dissolve the starchy material with 20 successively decreasing proportions of alkali solvent.

However, before this invention, when it has been attempted to produce in a jacketed 25 kettle such a vegetable glue suitable for gluing up veneers and the like, by such hot mixtures, the result has been that the glue has been "killed" or weakened so that it has not the strength and gluing qualities of mixtures made at ordinary temperatures or 30 "cold." The object of the present invention is to provide a method or process by which such a glue may be made with the application of heat, which requires less solvent, in 35 which "killing" or weakening the gluing properties of the starch mixture by overheating either locally or generally throughout the mass or by overcooking after the mixture has "come across" or the starch dissolved, is either eliminated entirely or reduced to a minimum so that it is negligible. 40 In the making of finishing glues, sizes, etc., it is not regarded as injurious to overcook or overheat or to boil the mixture of starch 45 and digesting agent, but in glue where the greatest adhesive power is desired, as in joinery, and the gluing up of veneers, this is found to be an important consideration and to secure a vegetable glue with such adhesive power and with suitable body and 50 spreading power it has been discovered that it is most undesirable to overheat the glue mixture as by boiling, or to overcook the

mixture by continuing the subjection thereof to a high temperature after the mixture 55 has come across. In fact the mixture should never attain the boiling, bursting or tumefying temperature and the temperature must not be maintained for a long time so high as to continue to an excessive degree the action 60 of the solvent on the glue. If the kettle be heated in the manner common in the mixing of sizes, etc., by admitting a strong current of steam to the kettle jacket the kettle becomes so intensely heated at all points that 65 the glue will become overheated, especially adjacent the inner walls of the kettle, so that the glue is likely to become "killed," which overcooking it is believed renders the starch mixture too low in degree of 70 mean polymerization, and consequently too fluid and too low in adhesive power. Also, if the application of a high temperature be continued after the mixture has "come across" the glue is similarly weakened. It 75 is therefore the main purpose of the present invention to check the action of the heat in such manner, and at such times, that the temperature of the batch will not reach the bursting temperature of the starch, and so 80 that the heat retained by the kettle will not cause overcooking after the mixture has come across or the starch dissolved. The word starch is used in its broad sense to mean any starchy or amylaceous material in 85 which raw starch or the more or less degenerated products thereof form the principal component, or other equivalent carbohydrate.

The accompanying drawing forming a 90 part of this specification illustrates an apparatus with which the invention may be carried out.

Referring to the drawing, 1 represents a suitable kettle having a jacket 2 and also 95 provided with any suitable stirring apparatus, not shown. The form of stirring apparatus shown in copending application Serial No. 612,181, filed March 4, 1911, is, however, preferred. 3 and 15 represent 100 steam supply pipes provided with valves 4 and 16, respectively, and connecting respectively with the pipes 7 and 8 which lead into the jacket 2, the first at the top and the second at the bottom of the jacket. 5 and 17 105 represent water supply pipes provided with

valves 6 and 18, respectively, and which also connect with the pipes 7 and 8 respectively. 9 represents an upright loop pipe having a valve at 11 therein, which pipe 9 connects at 15 one end with the pipe 8 and at its other end with exhaust pipe 14 at 18. A pipe 10 connects the two lower ends of the pipe 9, and is provided with a valve therein at 12. A pipe 19 connects the pipe 7 with pipe 9 and 20 is provided with a valve 20 therein. The jacket 2 is also provided with a pet-cock 21 at its upper end.

In carrying out the invention in one form, the required amount of water is placed in 15 the kettle with all the valves closed. The valves 4 and 12 are then opened to permit steam to enter the jacket and the water in the kettle is heated thereby, but not to over the bursting temperature of the starch, and 20 preferably not over 140° F. The valves 4 and 12 are then closed and when the temperature of the kettle has become equalized so that the temperature of the inner walls thereof is not too high, the starchy material 25 is added and stirred until thoroughly mixed with the water. Then the caustic soda solution or other digesting agent is added gradually with continued stirring. During this addition the valves 4 and 12 are 30 may be opened slightly to admit just enough steam to keep the temperature from falling too low until the mixture "comes across" or the starchy material is dissolved. When the mixture comes across the valves 4 and 12 are 35 closed and the valves 17 and 20 opened to admit cooler water in order to check the action of the heat to prevent overcooking after the starchy material has dissolved, the stirring of the batch being all the while preferably continued. The glue is then ready for 40 use or may be left to stand and again stirred and warmed if desired before using.

Or the invention in one form may be carried out by putting the starch and required 45 amount of water in the kettle and having it thoroughly mixed, and then the valves 6, 11 and 21 opened so as to nearly fill the jacket 2 with water up to the top of the loop 9. Then with continual stirring of the mixture 50 the valves 6, 11 and 21 are closed and the valves 16 and 20 opened and steam admitted to the lower part of the jacket so as to gradually heat the water in the jacket to the required degree. During this gradual heating 55 the solvent may be gradually added and when the mixture has come across the valves 16 and 20 are closed and the valves 5 and 11 opened to admit cooler water to the jacket so that the temperature of the batch is reduced 60 to about 120° F. to prevent overcooking of the glue after it has come across.

Although it is not preferred, the careful regulation of the heating may be obtained by opening the valves 4 and 12 and carefully admitting steam together with the 65

gradual addition of solvent and continual stirring of the mixture in the kettle great care being taken that the temperature at no part of the batch reaches the bursting temperature of the starch, and preferably not 70 over 150° F., and stopping the admission of the steam to check the action of the heat before the mixture has come across and at such time that the heat retained by the kettle will not produce overcooking after the mixture has come across. However, it is 75 preferred to check the action of the heat admitting cooler water to the jacket at such time that the heat retained by the kettle will not produce overcooking after the mixture has come across.

As above stated, the maximum temperature required varies with the amount of solvent used and it also varies with the kind of starch base and the kind of solvent used. 80 With high grade cassava starch preliminarily treated in accordance with description of United States Letters Patent 1,020,656 and 1% of caustic potash it is about 155° F. to 160° F., and decreases regularly as the amount of caustic is increased. With  $\frac{1}{2}$ % of caustic soda it is about the same and decreases in substantially the same manner with increase in the caustic soda. With 85 silicate of soda a larger percentage (about 18%) is required to produce really good results, and about 10% at 150° F. With salicylic acid, fairly good results can be obtained with 2% at 150° F.

Accordingly, the present invention is not 90 limited to precise temperatures or percentages of solvent, or kind of solvent, and many variations in these and other respects may be made without departing from the spirit and scope of the invention in its broader aspects.

Having fully and clearly described the improvements, what is claimed as new and desired to be secured by Letters Patent, is:

1. The process of making joiner's glue in a jacketed kettle from starch, water and solvent, which consists in stirring the glue mixture in the kettle and simultaneously heating the same by admitting a heating agent to the jacket but so that the temperature of the batch in the kettle will not reach the bursting point of the starch, and checking the action of the heating agent at such time that the heat retained will not cause overcooking of the glue after it has come 110 across or become dissolved.

2. The process of making joiner's glue in a jacketed kettle from starch, water and solvent, which consists in stirring the glue mixture in the kettle and simultaneously heating the same by admitting water to the jacket and injecting steam with the water to heat the latter but so that the temperature of the batch does not reach the bursting point of the starch, and checking the action 115 120 125 130

of the heat at such time that the heat retained will not cause overcooking of the glue after it has come across or become dissolved.

3. The process of making joiner's glue in a jacketed kettle from starch, water and solvent, which consists in stirring the glue mixture in the kettle and simultaneously heating the same by admitting a heating agent to the jacket but so that the temperature of the inner walls of the kettle will not reach the bursting point of the starch, and checking the action of the heat by admitting cooler water to the jacket at such time that the heat retained will not cause overcooking 15 of the glue after it has come across or become dissolved.

4. The process of making joiner's glue in a jacketed kettle from starch, water and solvent, which consists in stirring the glue mixture in the kettle and simultaneously heating the same by admitting water to the jacket and injecting steam into the water to heat the latter but so that the temperature of the batch does not reach the bursting 25 point of the starch, and checking the action of the heat by admitting cooler water to the jacket at such time that the heat retained will not cause overcooking of the glue after it has come across or become dissolved.

5. The process of making joiner's glue in a jacketed kettle from starch, water and solvent, which consists in stirring the glue mixture in the kettle and simultaneously heating the same by admitting a heating 35 agent to the jacket but so that the temperature of the batch will not be so great as to materially weaken the adhesive power of the glue for gluing up veneers, and checking the action of the heating agent at such time 40 that the heat retained will not cause over-

cooking of the glue after it has come across or become dissolved.

6. The process of making joiner's glue in a jacketed kettle from starch, water and solvent, which consists in stirring the glue mixture in the kettle and simultaneously heating the same by admitting a heating agent to the jacket but so that the temperature of the batch will not be so great as to materially weaken the adhesive power of 45 the glue for gluing up veneers, and checking the action of the heating agent by admitting cooler water to the jacket at such time that the heat retained will not cause overcooking 50 of the glue after it has come across or become dissolved.

7. The process of making joiner's glue in a jacketed kettle from starch, water and solvent, which consists in stirring the glue mixture in the kettle and simultaneously 55 heating the same by admitting water to the jacket and injecting steam with the water to heat the latter but so that the temperature of the batch will not be so great as to materially weaken the adhesive power of the 60 glue for gluing up veneers, and checking the action of the heat by admitting cooler water to the jacket at such time that the heat retained will not cause overcooking 65 of the glue after it has come across or become dissolved.

In testimony whereof, I have signed my name to this specification in the presence of two subscribing witnesses.

GERTRUDE S. PERKINS,  
*Executrix of Frank G. Perkins, deceased.*

Witnesses:

L. McMILLEN,  
M. McMILLEN.